

Nov. 28, 1944.

J. M. KENNEDY ET AL

2,363,973

## METHOD OF COPPER PLATING STAINLESS STEEL COOKING VESSELS

Filed July 8, 1939

7 Sheets-Sheet 1

Fig. 8.



Fig. 1.



### *Inventors:*

*James M. Kennedy,  
Arthur P. Knight,  
Harold J. Lee,*

Harold S. Lee,  
Wigmore Booth Townsend Miller & Weidner  
Attns.

Nov. 28, 1944.

J. M. KENNEDY ET AL.

2,363,973

## METHOD OF COPPER PLATING STAINLESS STEEL COOKING VESSELS

Filed July 8, 1939

7 Sheets-Sheet 2

Fig. 2.



*Inventors:*  
James M. Kennedy  
Arthur P. Knight,  
Harold J. Lee,  
by Emery Booth Townsend Muller & Weidner  
Attys

Nov. 28, 1944.

J. M. KENNEDY ET AL

2,363,973

## METHOD OF COPPER PLATING STAINLESS STEEL COOKING VESSELS

Filed July 8, 1939

7 Sheets-Sheet 3

Fig. 4.



*Inventors:*  
*James M. Kennedy,*  
*Arthur P. Knight,*  
*Harold J. Lee,*  
*by Emery Booth, Townsend Miller & Weidner*  
*Atty's.*

Nov. 28, 1944.

J. M. KENNEDY ET AL

2,363,973

METHOD OF COPPER PLATING STAINLESS STEEL COOKING VESSELS

Filed July 8, 1939

7 Sheets-Sheet 4

Fig. 5.



Fig. 6.



Inventors:  
James M. Kennedy,  
Arthur P. Knight,  
Harold J. Lee.

by Emery Booth, Townsend Miller & Weidner  
Hilys

Nov. 28, 1944.

J. M. KENNEDY ET AL

2,363,973

METHOD OF COPPER PLATING STAINLESS STEEL COOKING VESSELS

Filed July 8, 1939

7 Sheets-Sheet 5

Fig. 8.



Fig. 12.



Fig. 13.



Inventors:

James M. Kennedy  
Arthur P. Knight

Harold J. Lee.

By George Boot, Townsend Miller & Weidner  
Atty.

Nov. 28, 1944.

J. M. KENNEDY ET AL

2,363,973

METHOD OF COPPER PLATING STAINLESS STEEL COOKING VESSELS

Filed July 8, 1939

7 Sheets-Sheet 6

Fig. 9.



Fig. 10.



Inventors:  
James M. Kennedy,  
Arthur P. Knight,  
Harold J. Lee,  
by attorney Booth Townsend Miller & Weidner  
Attnys.

Nov. 28, 1944.

J. M. KENNEDY ET AL

2,363,973

METHOD OF COPPER PLATING STAINLESS STEEL COOKING VESSELS

Filed July 8, 1939

7 Sheets-Sheet 7

Fig. 11.



Inventors:

James M. Kennedy,  
Arthur P. Knight,  
Harold J. Lee.

by Harry Borth Townsend Miller & Weidner  
Attnys

## UNITED STATES PATENT OFFICE

2,363,973

## METHOD OF COPPER PLATING STAINLESS STEEL COOKING VESSELS

James M. Kennedy, Arthur P. Knight, and Harold J. Lee, Rome, N. Y., assignors to Revere Copper and Brass Incorporated, Rome, N. Y., a corporation of Maryland

Application July 8, 1939, Serial No. 283,432

15 Claims. (Cl. 204—34)

This application is a continuation-in-part of our co-pending application Serial Number 240,060, filed November 12, 1938, now Patent No. 2,272,609, which is a continuation-in-part of our co-pending application Serial Number 182,482, filed December 30, 1937, now abandoned.

Our invention relates to methods of making plated stainless steel articles, particularly but not exclusively to stainless steel cooking utensils having an electro-deposited coating of copper for distributing the heat.

The invention will be best understood from the following description of methods of making a cooking vessel, and description and accompanying drawings of the vessel and forms of apparatus for use in practice of the methods, the scope of the invention being more particularly pointed out in the appended claims.

In the drawings—

Fig. 1 is an elevation, with parts in section, of apparatus for use in preparing the surface of a stainless steel article for electro-depositing thereon a layer of copper or other metal;

Fig. 2 is a plan of the apparatus according to Fig. 1 with the motor omitted;

Fig. 3 is a section on the line 3—3 of Fig. 2 with parts omitted;

Fig. 4 is an elevation, with parts in section, of apparatus for use in electro-depositing a coating of copper or other metal on the article;

Fig. 5 is a plan of a fragment of the apparatus according to Fig. 4 with the motor and article, and support therefor, omitted;

Fig. 6 is a schematic diagram of electrical connections employed in connection with the apparatus according to Figs. 1 and 2;

Fig. 7 is a vertical diametric section of the bottom portion of the finished article, the thickness of the metals being exaggerated;

Fig. 8 is an elevation, with parts in section and parts omitted, of a modified form of apparatus for use in preparing the surface of a stainless steel article for electro-depositing thereon a layer of copper or other metal;

Fig. 9 is an elevation, with parts in section and parts omitted, of a modified form of apparatus for use in electro-depositing a coating of copper or other metal on the article;

Fig. 10 is a more or less diagrammatic representation, on an enlarged scale, of a fragment of the support and shield of Fig. 9;

Fig. 11 is a plan, with parts omitted, of a fragment of the apparatus according to Fig. 9;

Fig. 12 is a plan, on an enlarged scale, with parts

broken away, of the nozzle of the apparatus according to Figs. 9, 10 and 11; and

Fig. 13 is a section on the line 13—13 of Fig. 12.

The apparatus illustrated is particularly 5 adapted for electro-depositing a copper layer on the bottom surface of cooking vessels made of stainless steel, that is to say, iron, or iron-nickel alloy, containing sufficient chromium, say 6 to 25%, to make it stainless and corrosion resistant, and commonly small amounts of other metals present as impurities or added for improving the chemical and physical properties of the alloy. Although not limited thereto, an alloy containing 18% chromium and 8% nickel is very satisfactory for use in making cooking vessels according to the present invention.

It will be understood that stainless steel, although presenting a desirable material in respect to its resistance to the corrosive action of 10 foods, is unsatisfactory for cooking vessels such as frying pans, pots, and the like, for the reason that it is not only a relatively poor conductor of heat but conducts the heat non-uniformly in respect to different portions of its surface area 15 presented to the source of heat. For example, if it is attempted to cook batter in a stainless steel frying pan to produce a "pancake" no matter what cooking temperature is employed, the pancake will burn in spots before the portions between these spots will show any particular evidence of being cooked. To overcome this difficulty 20 it has been proposed to provide the under side of the bottom of a cooking vessel with a layer of copper or other material of high heat conductivity so as to distribute the heat over the 25 surface of that bottom. The apparatus and methods herein described are particularly useful in forming such a layer by electro-deposition on the bottom of a cooking vessel. It will be 30 understood, however, that the apparatus and methods described are not limited to use in connection with cooking vessels, but may be employed in connection with electro-depositing copper on any sort of stainless steel article.

45 In the practice of the method the surface to be plated is preferably first treated to clean it of grease. As suitable for this purpose applicants have found as satisfactory a solution which contains for each gallon of water 0.5 ounce sodium 50 hydroxide, 1.5 ounces sodium carbonate, and 4 ounces sodium silicate. The article may be allowed to stand in this alkaline solution for a short time until by observation or trial the grease is removed, after which it may be rinsed in water to remove all traces of the treating solution and

products of the reaction. However, if desired, any other known way and compound for "de-greasing" metal surfaces ordinarily may be employed for this purpose.

Applicants have found that it is impossible to electro-deposit an adhering coating of copper on stainless steel by any of the ordinary electro-plating methods. According to the invention, before electro-plating the cleaned surface of the article that surface is treated electrolytically to prepare it for the plating operation. As satisfactory for this purpose the article, or portion thereof on which the copper is to be electro-deposited, is made a cathode, and preferably an anode and then a cathode, in dilute acid. Applicants have found that in both the anodic and cathodic treatments best results will be secured by employing an electrolyte consisting of water containing about 30% by weight of sulphuric acid, to which solution preferably, but not necessarily, is added about 10% by weight of anhydrous sodium sulphate, and, for the electrolyte used for the cathodic treatment, preferably also sufficient substance such as sodium chloride to cause the electrolyte to contain about 0.05% by weight of chloride radical.

Either or both the sodium sulphate and chloride radical may be omitted. It has been found, however, that sodium sulphate improves the conductivity of the sulphuric acid electrolyte and also is electrolyzed to liberate sodium at the cathode when the article is made the cathode. This sodium reacts with the water to increase the amount of hydrogen liberated at the cathode, and thus cuts down the time necessary for cathodically treating the article. The chloride radical, it has been found, acts in the nature of a catalyst in respect to the effects produced when the article is a cathode, and when employed also acts to decrease the time necessary for cathodic treatment of the article. In practice the amount of sodium sulphate may be from about 5 to 15% of the electrolyte, and the range of the chloride radical from about 0.01 to 0.5% of the electrolyte.

The concentration of the sulphuric acid of the electrolyte employed in these preliminary treatments may vary from about 8.5 to 62% by weight. However, it has been found that the time necessary for treating the article for a given current density decreases as the concentration of sulphuric acid is increased from about 8.5 to 30% by weight, but no substantial decrease in time has been observed by increasing the sulphuric acid concentration above about 30% by weight.

When the article is made the anode it has been found that best results will be secured with current densities of from 300 to 350 amperes per square foot, although smaller and larger densities, say from 40 to 550 amperes per square foot of anode surface, may be employed. The total time of treating the article as an anode decreases as the current density is increased. This total time is such that the article is treated until etching of the surface begins, as shown by a "satin surface" just beginning to form on the article. Ordinarily the total time of this treatment will be from 30 to 45 seconds depending upon the current density employed within the range of from 40 to 550 amperes per square foot of anode surface.

Preferably much lower current densities are employed when the article is made the cathode. Preferably a current density of from 40 to 400 amperes per square foot of cathode surface is employed. The necessary time of treatment de-

creases with the current density, and ordinarily satisfactory results will be secured with a treatment of 1 to 3 minutes depending upon the current density. However, longer times of treatment are not precluded.

In treating the article anodically, as above described, plating off of its surface occurs slightly to roughen it, as evidenced by the production of a satin surface as above explained. This anodic treatment in some instances may be omitted, but without assurance of obtaining an adhering coating. If this omission is made, the surface may be roughened prior to cathodic treatment by other means, say by sand blasting, chemical etching, or the like.

When the article is made a cathode, hydrogen is evolved at its surface, which hydrogen acts as a deoxidizer and is believed also to form a film of hydrogen on said surface, protecting the surface while the article is being transferred to the plating bath and causing the plating to adhere to the surface. The time of this transfer and that which elapses before the plating operation is initiated should be kept at a minimum lest the hydrogen film be dissipated before the plating operation is initiated. It is necessary, so far as has been observed, to make the article a cathode to secure satisfactory results, and to make it a cathode last in respect to it being made the anode no matter how many times it may be made a cathode and an anode.

Electrolyte of the same composition preferably is employed when the article is both an anode and a cathode. Best results are secured when the electrolyte is kept at about room temperature when it is a cathode so as to minimize heating of the article and consequent dissipation of the hydrogen film. Preferably, to prevent the possibility of the article being treated cathodically in an electrolyte which has been deleteriously contaminated by employing it for treating the article anodically, these operations are performed in separate baths. After the satin surface forms when the article is treated anodically it may be immediately rinsed with water and placed in a second bath in which it is made the cathode. In such case only the bath in which the article is made the cathode need contain either the sodium sulphate or the chloride radical.

If the same bath is employed for both the anodic and cathodic treatments, alternations in the current may be made by use of a suitable pole changing device as, for example, the familiar double-throw two-pole switch, a resistance being thrown into circuit with the article when it is the cathode for reducing the current density to the desired value. Ordinarily but one alternation need be made, the article first being made an anode until the satin surface begins to form, and then made a cathode.

The article, after being cathodically treated as above described, is removed from the acid bath and placed in a plating bath. Preferably, so as not to increase the acidity of the plating bath, the treated surfaces of the article before being placed in the plating bath are washed with water, preferably at about room temperature, to free the surfaces of acid, and the article is placed in the plating bath before it dries. This washing operation may be performed by subjecting the article to a water spray or by immersing it in water. Preferably the article, if its shape permits, as would be the case with a cooking vessel, is axially rotated while being washed to subject all parts of its treated surfaces

to water, and is axially rotated when the washing is discontinued to throw off the excess water from its surfaces.

As above explained, the time which elapses between the cessation of the cathodic treatment of the article and the initiation of the plating operation on its treated surfaces should not be so prolonged as to permit material dissipation of the hydrogen film on the treated surfaces, and particularly the time the treated surfaces are exposed to the drying action of the air when wet with acid or water should be kept at a minimum to avoid dissipation of this film. Ordinarily to insure satisfactory results the total time which elapses should not exceed about half the necessary time of cathodic treatment, that is to say, if the article is treated cathodically for 1 minute should not exceed 30 seconds, or if treated cathodically for 10 minutes should not exceed 5 minutes, although 10 minutes' treatment in any ordinary case would be far in excess of that which is necessary. Further, it has been found that when the cathodically treated surfaces are placed in the plating electrolyte the latter acts to destroy the hydrogen film during the time which elapses before the plating current is established to initiate deposition. Therefore, the electrolyte to which the treated surfaces are exposed preferably is kept at about room temperature, say not over about 80° F. for an acid copper sulphate electrolyte, and the plating current established immediately upon the article being immersed in the electrolyte. Somewhat higher electrolyte temperatures, however, are not precluded, but the permissible elapse of time for establishing the plating current rapidly diminishes with the rise in temperature with decreased assurance of securing a strongly adhering electro-deposit, until with temperatures of about 140° F. the permissible time does not exceed about 20 seconds. It will therefore be understood that, in the sense the total time which may elapse between the cessation of the cathodic treatment and the initiation of electro-deposition, including the time for transferring the article and washing its cathodically treated surfaces, is limited to that which will not cause the electro-deposited coating to be non-adhering on account of dissipation of the hydrogen film or for other causes which would occur if the time were too prolonged, electro-deposition is initiated substantially immediately upon cessation of the cathodic treatment.

Best results it has been found will be secured in electro-plating the article by depositing thereon the copper in two distinct steps, the first involving the use of a high acid and low copper-content electrolyte, preferably sulphuric-acid copper-sulphate electrolyte, maintained at a relatively low temperature and with use of a plating current of relatively low density, and the second involving the use of a low acid and high copper-content sulphuric-acid copper-sulphate electrolyte maintained at a relatively high temperature and with use of a plating current of relatively high density. The first step is employed preferably to lay a thin, dense, strongly adhering layer or strike coating, and the second step to build up that coating to the desired thickness. Ordinarily, to make a coating that is bonded to the base metal strongly enough to withstand high temperatures and stresses to which a cooking vessel is subjected in use, the first coating preferably is just slightly more than a so-called "flash" coating. With the or-

dinary cooking vessel the total thickness of the coating, after the second coating is laid, will be at least 0.02 inch to secure satisfactory results. For vessels with thicker walls, say those exceeding 0.05 inch in thickness, the thickness of the copper coating ordinarily should be increased proportionally to secure best results.

As a suitable example of the plating method, but without limitation thereto, the thin preliminary coating may be electro-deposited employing a 20% (by weight) sulphuric acid electrolyte containing about 10% (by weight) copper sulphate. However, from 5 to 40% (by weight) sulphuric acid may be employed with 5 to 20% (by weight) copper sulphate, the amount of copper sulphate varying inversely with the amount of acid. Preferably, in laying this coating, the article is rotated, or motion between it and the electrolyte otherwise caused.

With these electrolytes for the preliminary copper layer a current density of up to 100 amperes per square foot of cathode surface may be employed, the anode preferably being soluble as, for example, being formed of copper. Higher current densities, say up to 300 amperes per square foot of cathode surface, and high percentage copper sulphate electrolytes, could be employed, but it would be necessary under such conditions strongly to agitate the electrolyte to keep down "burning" of the copper layer, and such agitation would be liable to admit air and destroy that property of the stainless steel surface which enables the coating to be placed upon it.

Under the above conditions the preliminary coating is formed in from 20 seconds to 3 minutes depending upon the current density and the copper sulphate concentration of the electrolyte. The coating is dense and of fine grain, and strongly adheres to the stainless steel so as to be in substance integral therewith in the finished article.

Although it is preferred to employ an acid copper sulphate electrolyte for the preliminary strike coating, other suitable electrolyte may be employed as, for example, an aqueous copper cyanide electrolyte, say one containing 3 ounces (by weight) of copper per gallon in the form of copper sodium cyanide, with 0.5 to 3 ounces (by weight) of free sodium cyanide per gallon to increase the conductivity of the electrolyte and provide anode corrosion. With the copper cyanide electrolytes a slightly higher temperature, not less than 110° F., must be employed.

The preliminary step of electro-plating could be continued to lay a coating of the desired thickness in the finished article, but would involve such time as to be economically prohibitive. Consequently, for laying the remainder of the coating, preferably the article is transferred from the bath just mentioned to a second bath without permitting it to dry, or without rinsing it if the preliminary coating is deposited from a copper sulphate electrolyte. It has been found that, to secure good results, if the article is accidentally permitted to dry at this stage of the process it will be necessary thoroughly to clean the copper surface with an acid preparatory to continuing the plating operation.

Preferably the second bath consists of about 10% (by weight) sulphuric acid electrolyte containing about 20% (by weight) copper sulphate. The sulphuric acid may, however, range from 5 to 15%, and the copper sulphate from 15 to 25% inversely with the amount of sulphuric acid. Preferably the electrolyte also contains from 2 to

4 ounces per gallon of aluminum sulphate to give a smoother surface to the finished copper coating.

The above mentioned electrolyte employed for laying the final copper coating is maintained preferably at a temperature of about 130° F. to increase the rate of deposition. Temperatures up to 150° F. may be employed, but preferably the temperature is not raised to above 130° F. to prevent the plating from becoming too coarse.

Current densities up to about 500 amperes per square foot may be employed, and for the higher ranges of current density preferably not only is the work rotated, or motion between it and the electrolyte otherwise caused, but the electrolyte is strongly agitated as, for example, by introducing into it a jet of air, or by pumping electrolyte against either or both the anode and cathode. It has been found that by relatively moving the work and electrolyte and agitating the latter a smoother coating is laid for a given current density, and that higher current densities may therefore be employed under these conditions.

The anode of the cell employed in this second step preferably is a soluble copper anode which, it has been found, imparts better physical properties to the coating than does an insoluble anode.

Copper, plated as above described, it has been found, will adhere to the treated stainless steel even when plated on sheets and the same are bent back and forth at right angles until they fracture. In this connection it will be understood that severe flexing occurs in a cooking vessel when the bottom is heated and permitted to cool. Further, up to ordinary cooking temperatures, say 650° F., it has been found that the coating in respect to its bond with the stainless steel is strongly resistant to heat, and will not loosen under such conditions. It is dense and hard, and admirably withstands the rough treatment to which it is subjected when scoured by the housewife to clean it.

It is possible to place the article after being cathodically treated in the cell having the anode and plating bath for performing the final plating operation described above, and omit the operation of forming the flash coating as a preliminary step, but only with some sacrifice of the excellence of the results secured and with less assurance of uniformly satisfactory results being obtained. In such case the coating will be much coarser, and less assurance will be had that the coating will adhere. Further, in such case, extreme care must be taken that on account of the rather high temperature of the electrolyte the plating current is established without delay when the cathodically treated article is immersed in it, and an attempt to avoid this difficulty by lowering the temperature of the electrolyte will result in materially decreasing the rate of deposition. Still further, on account of the high current densities that would be employed in this case it would be necessary strongly to agitate the electrolyte to prevent burning of the copper, and such agitation would result in the possibility of admitting air against the cathodically treated surface, thus reducing the assurance that a good adherence of the coating would be obtained. In these connections it will be understood that preliminary rather slowly laying a strike coating with an electrolyte of low temperature and concentration by use of a plating current of low density not only insures strong adherence of the coating because of these factors but lays a dense smooth coating, which smooth-

ness, it will be understood by those skilled in the art, is imparted to the exposed surface of the final coating when it is deposited at a more rapid rate.

5 Figs. 1 and 2 illustrate one form of apparatus for use in anodically and cathodically treating the surface of a stainless steel cooking vessel on the bottom and adjacent portions of which is to be electro-deposited the layer of copper or other good heat conductive material.

10 Referring to Figs. 1 and 2, the body 1 of electrolyte is contained in a suitable receptacle 3 as, for example, a lead pot, herein shown as supported by a table top 5 of wood, the table top having an opening 7 through which the pot extends for allowing the circumferential flange 9 at the top of the pot to rest upon the top of the table.

15 As shown in Figs. 1 and 2, supported in the pot 3 is a cup-shaped electrode, preferably of insoluble material such as lead, having the bottom wall 11 and side walls 13, the bottom wall being provided with a plurality of spaced perforations 15 distributed thereover, and the side walls being provided with a lower circumferential row of perforations 17 and an upper row of perforations 19, the bottom of the perforations 19 being at about the level of the electrolyte. As shown, the electrode is supported by a plurality of straps, made for example of lead, having the vertical portions 21 joined to the upper edge of the electrode and horizontal portions 23 which rest upon the flange 9 of the pot. Conveniently, one or more of these straps is connected to a lead 25 from one terminal of the source of plating electromotive force.

20 30 35 As illustrated, at one side of the pot the table top 5 supports a vertical standard 27 on which is slidably mounted an arm 29 adapted to be secured to the standard in adjusted positions vertically thereof by a set screw indicated at 31. At one end this arm 29 carries the vertical post 33, preferably of insulating material, to which is detachably secured the casing 35 of an electric motor, the rotary metal shaft 37 of the motor projecting vertically downward from the motor casing. 40 45 50 55 This shaft extends through an elongated stationary metal sleeve 39 in contacting relation with the walls thereof, the sleeve being carried by a metal arm 41 in electrical communication therewith. As shown, the arm 41 has a vertical portion 43 which is rigidly joined to the arm 29 in insulated relation thereto and is placed in electrical communication with the other terminal of the source of plating electro-motive force by a lead 45 so that the shaft 37 of the motor serves as part of the conductor leading to the cooking vessel V being treated.

60 65 70 As shown (Figs. 2 and 3), for joining the vertical portion 43 of the arm 41 to the arm 29, the portion 43 is provided at opposite sides thereof at its upper end with a pair of projections 47 embracing the arm 29. A pair of bolts 49, extending through aligned openings in the projections 47 and arm 29, serve to secure the latter and the vertical portion 43 of the arm 41 in assembled relation, the two being insulated from each other and from the bolts by suitable insulation 51 and 53. These bolts are employed also to secure the bases 55 of the terminal lugs 57 on the end of the lead 45 in electrical communication with the vertical portion 43 of the arm 41, as will be clear from Fig. 3.

75 As illustrated, detachably joined to the end of the metal shaft 37 of the motor, by means of the metal sleeve 59 and set screws 61, is a second

metal shaft 63. This latter shaft carries at its lower end, in electrical communication therewith, a chuck for supporting the cooking vessel V. As shown, the chuck, which preferably is formed of resilient sheet copper, has a bottom 65, to which the shaft 63 is joined, and has side walls formed with V-shaped splits 67 to form a circumferential series of spaced resilient prongs 69, the latter engaging the lower portions of the side walls of the cooking vessel for supporting it and placing it in electrical communication with the shaft 63.

In operation, when the motor is energized the vessel V is rotated. Satisfactory results will be secured in the practice of the above described method when the speed of rotation is such as to give a linear speed at the outer periphery of the vessel corresponding to 150 to 300 R. P. M. for a vessel 7 inches in diameter. Other speeds, however, are not precluded.

The bottom of the vessel, which in practice may be spaced from the bottom of the cup-shaped electrode a distance of from about  $\frac{1}{2}$  to  $\frac{3}{4}$  inches, when rotated, forms with that electrode a centrifugal pump which draws the electrolyte through the perforations 15 at the center portions of the cup-shaped electrode and forces it out of the perforations 17 and out of the perforations 15 adjacent the periphery of the electrode, thus circulating the electrolyte rapidly in contact with the bottom of the vessel. A certain portion of the electrolyte flows upward to discharge through the perforations 19, which latter serve as an overflow to maintain approximately constant the level of the electrolyte in the annular space between the vertical walls of the vessel and the cup-shaped electrode. By this means, for a purpose herein-after described, the portions of the side walls of the vessel adjacent its bottom are treated.

The circuit arrangement used in connection with the apparatus just described, when employed for treating the vessel as both a cathode and an anode, is schematically illustrated in Fig. 6. Referring to Fig. 6, the leads 71 from a source of plating electromotive force are connected to the center terminals of a double-throw two-pole switch schematically indicated at 73. The upper terminals of this switch are connected by leads 75 and 77 to the cup-shaped electrode 11, 13 and the vessel V respectively. The lower right hand terminal of the switch is connected by a lead 79 to the lead 75, and the lower left hand terminal to the lead 77 through a variable ohmic resistance 81. By this arrangement, when the switch 73 is thrown to connect the leads 71 to the upper terminals of the switch, a high plating current will be passed through the bath, under which conditions the vessel V is the anode. When the switch is thrown to connect the leads 71 to the lower terminals of the switch to make the vessel V the cathode the resistance 81 is thrown into circuit to cut down the plating current below that which it was when the vessel was the anode.

The depth the cooking vessel V is immersed in the electrolyte can be readily adjusted by moving the arm 29 up and down the standard 27. Preferably a stop collar 83, which may be secured to the standard 27 in adjusted positions by use of a set screw 85, is provided, so that by causing the arm 29 to rest against the collar when the arm is in its lower position all vessels V of similar size will be immersed in the electrolyte the same depth. At the completion of the operation the set screw 31 may be loosened and the arm 29 raised to move the vessel out of the electrolyte, 75

thus permitting the vessel to be readily slipped out of engagement with the clutch on the end of the shaft 63.

Another form of apparatus for use in the preliminary treatment of the stainless steel vessel is shown in Fig. 8. This apparatus is exactly like that illustrated in Figs. 1, 2 and 3, except that a flat anode 139 having the perforations 15 is employed instead of a cup-shaped anode, the anode being supported by straps 141 similar to the straps 21 hereinbefore mentioned. Except that in some instances a slightly greater time is required for the treatment when employing the flat electrode, equally efficacious results will be secured with it as compared to those obtained with the cup-shaped electrode, with the advantage that by making the flat electrode of large diameter it is adaptable for use with a wider range of diameters of vessels than is the cup-shaped electrode.

One form of apparatus for electro-depositing the copper is illustrated by Figs. 4 and 5. This apparatus is similar to that heretofore described in respect to the support for the motor and vessel V, and the description of that part of the apparatus need not therefore be repeated.

As shown (Figs. 4 and 5), this last mentioned apparatus comprises a tank 87 formed, for example, of iron lined with insulating material 89 such as rubber. Along one edge of the tank, in insulated relation thereto, is shown a bus-bar 91 serving as one terminal of the source of plating electromotive force, the other terminal of which is constituted by the lead 45 in electrical communication with the vessel V.

Connected to the bus-bar, in electrical communication therewith, is an anode support, preferably in the form of a copper casting having a coating 93 of lead to protect it from corrosion and from plating off of its surface. As shown, this support comprises a horizontal portion 95 which rests upon and is bolted by means of bolts 97 to the bus-bar 91 in electrical communication therewith. Connected to the horizontal portion 45 is a vertical portion 99 which projects downward into the electrolyte tank and carries a horizontal portion 101 to the outer end of which is secured a soluble anode 103 of copper or other metal to be plated on the vessel V. As shown, a disk 105, 50 of relatively strong metal such as copper, has soldered thereto a disk 107 of lead which is "burned" to the lead lining 93 of the anode support. The soluble anode 103 on its lower side is provided with a recess 109 which receives the disk 105 to which it is detachably secured in electrical communication therewith by screws 111.

As illustrated, the anode 103 is provided with a plurality of spaced perforations 113 through which electrolyte is drawn into the space between the anode and vessel V when the latter is rotated.

The anode 103 and its supporting disks 105 and 107 as shown in Figs. 4 and 5 are provided with aligned central perforations 114 into which extends the end of a vertical pipe 115 formed of lead or other material inert with respect to the electrolyte. This pipe leads from a box 117, formed of similar material, which box is supplied with air under pressure by a pipe 119 of rubber or other material inert with respect to the electrolyte, the amount of air admitted to the box being controlled, and when desired the air being cut off, by a valve not shown. The box, as shown, is supported by a bracket 121 of lead or other material inert with respect to the electrolyte car-

ried by the tank preferably in insulated relation thereto. At the top of the pipe 115 is a small hole 125, say one about  $\frac{1}{16}$  of an inch in diameter, which discharges the air in an upward direction toward the vessel V. This air causes agitation of the electrolyte and eliminates the possibility of the existence of quiescent spots in the electrolyte adjacent the center of the bottom of the rotating vessel, which spots, if they existed, might cause "burning" of the copper being deposited. Further agitation of the electrolyte is caused by the same being drawn through the perforations 113 and 114 of the anode when the vessel is rotated, and being discharged outward from the space between the anode and the vessel at the periphery of the anode. Still further agitation of the electrolyte is caused by providing the top of the box 117 with fine holes 127, say about  $\frac{1}{16}$  of an inch in diameter, through which air is discharged.

It will further be understood that the temperature of the electrolyte may be controlled by varying the amount of air admitted. It will also be understood that by moving the electrolyte and vessel relative to each other a scouring effect is produced which improves the physical properties of the copper by making it of fine grain. In laying the preliminary "strike" coating of copper in the above described method it will be understood that the air supply is interrupted to prevent oxidation of the treated stainless steel surface and thus cause the copper to adhere as hereinbefore explained.

It will be observed from Fig. 1 that the extreme lowermost portions of the side walls 129, and curved corner portions 131 which join the side walls to the bottom 133 of the cooking vessel V, are treated by the preliminary operation to permit their being electro-plated with copper. As will be clear from Fig. 4, the corner portions 131 and adjacent side wall portions are more remote from the anode 103 than is the bottom 133. In consequence of this, the copper coating 135 laid is of gradually diminishing thickness as it extends from the bottom 133 of the vessel over the corner portions 131 and such of the adjacent side wall portions thereof, if any, as may be subjected to deposition, until the coating merges at 137 with the stainless steel surface preferably at about where the corner portions merge into the side walls, as is illustrated in Fig. 7, or slightly above or below it, the rate of diminution of thickness for different increments of length on the profile of the vessel being roughly the rate of decrease in current density for those increments as influenced by the rate of increase in the distance of those increments from the anode. As shown, however, Fig. 7 is more or less approximate, and in practice the edge of the coating may be positioned somewhat differently from there shown, as desired and depending upon the depth of immersion of the article and its speed of rotation during the plating operations. The coating described provides the vessel with a copper coating on its lower exterior surface portions, the edges of which coating are free from projecting corners, and thus not only improves the appearance of the article but eliminates any shoulders or cracks at which peeling off of the copper might start by mechanical action, or at which grease and dirt might accumulate or enter to start peeling by corrosive action of the copper. Any slight irregularities which may exist at the edges of the copper layer as a result of the plating op-

eration may ordinarily be readily removed by a slight buffing operation. It will also be observed that rotating the vessel eliminates any variations in the effective lengths of current paths from the anode to different portions of the vessel having a symmetrical relation with each other, and that as a consequence the coating, in respect to thickness, and at its edges, is laid substantially symmetrically with respect to the vessel.

10 Conveniently the article is immersed in the sulphuric acid electrolyte during the preliminary treatment a slightly greater distance than in the copper bearing electrolytes so as to insure that no untreated surfaces will be subjected to deposition. In depositing the copper, the electrolyte tends slightly to creep up the walls of the rotating vessel, say about  $\frac{1}{16}$  of an inch above the normal electrolyte level, in the form of a rather attenuated film of diminishing thickness 20 as it extends above that level, which film also aids in causing the copper deposit to merge into the surface of the stainless steel because the rate of deposition in this film is very small.

If desired, the copper deposit may be coated 25 with a thin electro-deposit of nickel, chromium or other tarnish and corrosion resistant metal to protect the copper against corrosion and pitting. This final coating may be applied in the usual manner employed in the art.

30 Another form of apparatus for plating the copper is shown in Figs. 9 to 13. In this latter form of apparatus the anode takes the form of a flat copper disk 143 opposed to the bottom surface of the vessel V in coaxial relation therewith.

35 As illustrated, the anode is formed with a center opening 145 which receives a boss 147 projecting upwardly from the upper side of the terminal portion 149 of a support, this terminal portion having a flat upper surface in which the bottom 40 side of the anode rests.

As shown, the anode 143 is secured to the support by means of the nozzle illustrated in Figs. 12 and 13. This nozzle, which is formed of hard rubber or other suitable insulating material, as 45 shown comprises a flat head 151 and an exteriorly screw-threaded shank 153, the latter being screwed into a screw-threaded perforation 155 (Fig. 9) which extends through the boss 147 and terminal portion 149 of the support, a suitable 50 washer or washers 157 of metal such as lead being interposed between the head 151 and the upper surface of the anode. By reason of this construction no plating off of the anode beneath the head 151 can occur, and that portion of the 55 anode therefore remains of the same thickness as the plating operations continue and the anode therefore will not become loose but will always remain firmly clamped to and in electrical contact with the upper surface of the terminal portion 149 of the support. Also the head 151 being 60 of insulating material causes the plating current to follow a longer path from the anode to the axial portions of the cathode surface than to adjacent portions thereof, the advantage of 65 which will hereinafter be described.

The terminal portion 149 of the support for the anode 143 is carried at the end of an arm 159, the support being otherwise like the support 85, 99, 101 heretofore described and being 70 in electrical communication with the bus-bar 81.

As illustrated, the opening 161 in the shank 153 of the nozzle communicates with the wide flaring radial passages 163 formed in the head 151, these passages being separated by narrow 75 partitions 164 distributed circumferentially of

the head. The opening 161 also communicates with a plurality of small diameter openings 165 opening on the upper side of the head. As a result of this construction electrolyte supplied to the nozzle will be discharged radially from the passages 163 through the space between the anode and bottom surface of the cooking vessel in substantially all directions, and from the openings 165 upwardly against said surface adjacent its axial portion.

In this modification, for supplying the nozzle with electrolyte, screw-threaded into the lower end of the opening 155 of the terminal portion 149 of the support is an elbow 167 (Fig. 9) to which is secured the end of a rubber hose 169 supplied with electrolyte from a manifold 171 at the exterior of the tank 89, this manifold having an outlet nipple 173 to which the opposite end of the hose is secured. Conveniently the hose is provided with a pinch cock 175, or other suitable valve is provided for regulating the flow of electrolyte through the hose so that the amount thereof which discharges from the nozzle may be readily controlled.

As shown in Fig. 11, electrolyte is drawn from one end of the tank 89 through a pipe 177 by means of a suitably driven pump 179. This pump, by way of the pipe connection 180, forces the electrolyte through a suitable filter 181, and from the latter into the communicating manifold 171, the manifold extending lengthwise of the tank and being provided with an outlet nipple 173 for each of the units for plating the vessels V. In practice the pinch cocks may be set to discharge in the order of five gallons of electrolyte per minute through each nozzle.

The electrolyte which is discharged through the openings 165 of the nozzle eliminates the possibility of quiescent spots in the electrolyte at the axial portion of the bottom of the rotating vessel, which spots, if they existed, might cause "burning" of the copper being deposited. The electrolyte so discharged and that discharged radially of the anode from the passages 163 of the nozzle cause agitation of the electrolyte to prevent, in conjunction with the rotation of the vessel, "burning" of the copper when the high current density is employed. It will be understood, however, that ordinarily it will be unnecessary to supply electrolyte through the nozzle when the preliminary strike coating is being deposited on account of the low current density employed for that operation.

As illustrated in Figs. 9, 10 and 11, there is interposed between the anode 143 and the cathode constituted by the vessel V a shield indicated in its entirety at 183. This shield is of annular shape having a central opening 185 coaxial with the axis of rotation of the vessel. The shield conveniently may be formed of a flat steel plate 187 covered with a layer 189 of rubber or other compound inert with respect to the electrolyte. The shield as shown is supported by a ring 191 formed with a plurality of integrally projecting lugs 193 on which the shield removably rests, the outer periphery of the shield preferably snugly fitting the interior peripheral portion of the ring. As illustrated, the ring is formed integrally with a vertically extending rod 195 which at its upper end is joined to a collar 197 slidably mounted on the vertical post 199 carried by the tank. By use of the set screw 201 the collar and hence the shield may be adjusted into different vertical positions. Preferably the rod, ring and lugs are coated with a layer 203 of

rubber or other compound inert with respect to the electrolyte.

By use of the shield, which may also be employed in situations where air is admitted through the anode into the space between the latter and the bottom surface of the vessel, as in the apparatus illustrated in Fig. 4, the path of travel of the plating current from the anode to the cathode constituted by the vessel progressively increases from points opposite the inner peripheral edge of the annular shield to the edges of the surface being plated. Hence, as the ohmic resistance increases with the length of path of travel of the current, the value of the current and consequent rate of deposition progressively diminish from points opposite the inner peripheral edge of the shield to the edges of the surfaces being plated as compared to what they would be were the shield omitted. It has been found that when the anode is not of materially smaller diameter than the surface being plated the deposit in absence of the shield tends to be heaviest at the edge or corner of the cathode. For example, if the diameters of the cathode and anode are as shown in Fig. 9, in absence of the shield the deposit at the rounded corners of the bottom of the vessel would be of greater thickness than at adjacent portions of the bottom. The shield by diminishing the rate of plating at the corners eliminates this effect and permits various size diameter vessels to be plated with the same large diameter cathode by substituting different shields and to a lesser extent by adjusting the position of the shield vertically. For a given vessel the closer the shield is to it the thinner the deposit will be at the corner, and therefore by properly positioning the shield the thickness of the deposit at the corner may be regulated. The shield also causes the deposit at the rounded corner to be of decreasing thickness as the edge of the deposit is approached, and by its use the deposit at the edge thereof can be made approximately a feather edge merging into the side wall of the vessel. To secure this effect without the presence of the shield the anode must be of proper smaller diameter than the vessel.

It has also been found that the head 151 which holds the anode in place acts to diminish the plating current and consequent rate of deposition at the axial portion of the bottom of the vessel. If the cathode extended over the space occupied by the head it has been found that the deposit would tend to be somewhat thicker than at the intermediate portions of the radial of the bottom surface of the vessel. The head therefore acts to increase the length of path of the plating current from the anode to points opposite the head, and in this respect acts like the shield.

It will be understood that within the scope of the appended claims wide deviations may be made from the forms of the invention herein described without departing from the spirit of the invention.

We claim:

1. The method of coating the bottom and adjacent side wall surfaces of a stainless steel cooking vessel with a strongly adhering layer of copper which comprises preliminarily treating said surfaces to roughen them, subjecting the roughened surfaces to electrolytically released hydrogen without depositing metal on them by immersing the bottom portions only of the vessel in a non-metal bearing dilute aqueous sulphuric

acid and while axially rotating the vessel making it a cathode; removing the vessel from said acid at the completion of the cathodic treatment and substantially immediately immersing said bottom portions in an aqueous sulphuric acid copper bearing electrolyte and initiating electro-deposition of copper thereon by making the vessel a cathode and while axially rotating said vessel electro-depositing on the cathodically treated surfaces a strike coating of copper with a plating current not exceeding 100 amperes per square foot of cathode surface; and then transferring said vessel to and immersing said bottom portions in a high copper content aqueous sulphuric acid electrolyte and while axially rotating said vessel electro-depositing on said strike coating a relatively thick layer of copper with a plating current of greater density than the first mentioned plating current.

2. The method of coating the bottom and adjacent side wall surfaces of a stainless steel cooking vessel with a strongly adhering layer of copper which comprises preliminarily treating said surfaces to roughen them, subjecting the roughened surfaces to electrolytically released hydrogen without depositing metal on them by immersing the bottom portions only of the vessel in a non-metal bearing dilute aqueous sulphuric acid and while axially rotating the vessel making it a cathode; removing the vessel from said acid at the completion of the cathodic treatment and substantially immediately immersing said bottom portions in an aqueous copper bearing electrolyte and initiating electro-deposition of copper thereon by making the vessel a cathode, and while rapidly axially rotating said vessel electro-depositing on the cathodically treated surfaces a strike coating of copper with a plating current not exceeding 100 amperes per square foot of cathode surface; and while rapidly axially rotating the vessel with said bottom portions immersed in a high copper content aqueous sulphuric acid electrolyte electro-depositing on said strike coating a relatively thick layer of copper by use of a plating current of greater density than the first mentioned plating current.

3. The method of coating the bottom and adjacent side wall surfaces of a stainless steel cooking vessel with a strongly adhering layer of copper which comprises preliminarily treating said surfaces to roughen them, subjecting the roughened surfaces to electrolytically released hydrogen without depositing metal on them by immersing the bottom portions only of the vessel in a non-metal bearing dilute aqueous sulphuric acid and while axially rotating the vessel making it a cathode; removing the vessel from said acid at the completion of the cathodic treatment and substantially immediately immersing said bottom portions in an aqueous copper bearing electrolyte to a lesser depth than they were immersed to treat them cathodically in said acid and initiating electro-deposition of copper thereon by making the vessel a cathode, and while rapidly axially rotating said vessel electro-depositing on the cathodically treated surfaces a strike coating of copper with a plating current not exceeding 100 amperes per square foot of cathode surface; and while rapidly axially rotating the vessel with said bottom portions immersed in a high copper content aqueous sulphuric acid electrolyte electro-depositing on said strike coating a relatively thick layer of copper by use of a plating current of greater density than the first men-

tioned plating current, in which latter electrolyte said strike coating is immersed to no greater depth than said bottom portions were immersed while the strike coating was being deposited.

5. The method of electro-depositing a strongly adhering layer of copper on the lower exterior surface portions including the bottom of a stainless steel cooking vessel or the like so formed that said surface portions are surfaces of revolution which comprises roughening said surface portions and afterward subjecting them to electrolytically released hydrogen without depositing metal on them by making them a cathode in a non-metal bearing aqueous sulphuric acid electrolyte, substantially immediately upon completion of such cathodic treatment subjecting said surface portions to electro-deposition of the copper layer, the electro-deposition of said layer comprising making the vessel a cathode with the axis of said surface portions positioned vertically and with said lower surface portions partially immersed in an aqueous sulphuric acid copper bearing electrolyte in spaced relation to an anode from which the current travels along longer paths to the edge portions of said surface portions than to intermediate portions thereof, the lengths of said paths at said edge portions progressively increasing as the outer edges thereof are approached, and relatively rapidly rotating said vessel about said axis while depositing thereon a copper coating and at such speed as to draw an attenuated film of electrolyte up the edge portions of the vessel above the normal electrolyte level, whereby said coating is symmetrically deposited with relation to said axis and at said edge portions is of gradually decreasing thickness as the edges of said coating are approached and said coating at its edges has a portion of material width and attenuated thickness substantially merging into said surface portions.

- 40 5. The method of coating the bottom surfaces of a stainless steel cooking vessel with a strongly adhering layer of copper which comprises preliminarily roughening said surface, making the roughened surface a cathode in a non-metal bearing aqueous sulphuric acid electrolyte to subject it to electrolytically released hydrogen without depositing metal thereon, and removing it from said acid electrolyte upon the completion of the cathodic treatment and substantially immediately immersing it in an aqueous copper bearing electrolyte and initiating electro-deposition of copper thereon.

- 45 6. The method of coating the bottom surface of a stainless steel cooking vessel with a strongly adhering layer of copper which comprises etching said surface by making it an anode in a non-metal bearing aqueous sulphuric acid electrolyte, afterward making the etched surface a cathode in a non-metal bearing aqueous sulphuric acid electrolyte to subject it to electrolytically released hydrogen without depositing metal thereon, and removing it from said acid electrolyte upon the completion of the cathodic treatment and substantially immediately immersing it in an aqueous sulphuric acid copper bearing electrolyte and initiating electro-deposition of copper thereon.

- 50 7. The method according to claim 6 in which the stainless steel surface is made an anode for etching it in the same non-metal bearing aqueous sulphuric acid electrolyte as that in which it is made a cathode for subjecting it to hydrogen.

- 75 8. The method of coating the bottom surface of a stainless steel cooking vessel with a strongly

adhering layer of copper which comprises etching said surface by making it an anode in an aqueous sulphuric acid electrolyte, removing said surface from said electrolyte and substantially immediately rinsing it with water and immersing it in a second non-metal bearing aqueous sulphuric acid electrolyte, making the etched surface a cathode in the latter electrolyte to subject it to electrolytically released hydrogen without depositing metal thereon, and removing it from said second electrolyte upon the completion of the cathodic treatment and substantially immediately rinsing it with water and immersing it in an aqueous copper bearing sulphuric acid electrolyte, and when so immersed substantially immediately making it a cathode to initiate electro-deposition of copper thereon.

9. The method of coating a stainless steel surface of a cooking vessel with a strongly adhering layer of copper which comprises roughening said surface, making the roughened surface a cathode in a non-metal bearing aqueous sulphuric acid electrolyte to subject it to electrolytically released hydrogen without depositing metal thereon, removing the vessel from said acid electrolyte upon the completion of the cathodic treatment and substantially immediately immersing it in an aqueous sulphuric acid copper sulphate electrolyte having, by weight, 10 to 40% sulphuric acid and 5 to 20% copper sulphate with the amount of sulphuric acid greater than the amount of copper sulphate and initiating electro-deposition of copper thereon by use of a plating current not exceeding 100 amperes per square foot of cathode surface; and, after deposition of a strike coating of copper thereon, electro-depositing a relatively thick layer of copper on said strike coating by use of an aqueous sulphuric acid copper sulphate electrolyte having, by weight, 5 to 15% sulphuric acid and 15 to 25% copper sulphate but with the amount of sulphuric acid less than the amount of copper sulphate and a plating current of greater density than the first mentioned plating current but not exceeding 500 amperes per square foot of cathode surface.

10. The method of coating a stainless steel surface of a cooking vessel with a strongly adhering layer of copper which comprises roughening said surface, making the roughened surface a cathode in a non-metal bearing aqueous sulphuric acid electrolyte to subject it to electrolytically released hydrogen without depositing metal thereon, removing the vessel from said acid electrolyte upon the completion of the cathodic treatment and substantially immediately immersing it in an aqueous sulphuric acid copper sulphate electrolyte not materially above room temperature and having, by weight, 10 to 40% sulphuric acid and 5 to 20% copper sulphate with the amount of sulphuric acid greater than the amount of copper sulphate and initiating electro-deposition of copper thereon by use of a plating current not exceeding 100 amperes per square foot of cathode surface; and, after deposition of a strike coating of copper thereon, electro-depositing a relatively thick layer of copper on said strike coating by use of an aqueous sulphuric acid copper sulphate electrolyte having, by weight, 5 to 15% sulphuric acid and 15 to 25% copper sulphate but with the amount of sulphuric acid less than the amount of copper sulphate and a plating current of greater density than the first mentioned plating current but not exceeding 500 amperes per square foot of cathode surface.

11. The method of coating a stainless steel surface of a cooking vessel with a strongly adhering layer of copper which comprises etching said surface by making it an anode in an aqueous sulphuric acid electrolyte, making the etched surface a cathode in a non-metal bearing aqueous sulphuric acid electrolyte to subject it to electrolytically released hydrogen without depositing metal thereon, removing the vessel from the last mentioned acid electrolyte upon the completion of the cathodic treatment and substantially immediately immersing it in an aqueous sulphuric acid copper sulphate electrolyte not materially above room temperature and having, by weight, 10 to 40% sulphuric acid and 5 to 20% copper sulphate with the amount of sulphuric acid greater than the amount of copper sulphate and initiating electro-deposition of copper thereon by use of a plating current not exceeding 100 amperes per square foot of cathode surface; and, after deposition of a strike coating of copper thereon, electro-depositing a relatively thick layer of copper on said strike coating by use of a second aqueous sulphuric acid copper sulphate electrolyte and a plating current of greater density.

12. The method of preparing a stainless steel surface of a cooking vessel for receiving a relatively thick, strongly adhering layer of electro-deposited copper which comprises roughening said surface, making the roughened surface a cathode in a non-metal bearing aqueous sulphuric acid electrolyte to subject it to electrolytically released hydrogen without depositing metal thereon, and removing the vessel from said electrolyte upon the completion of the cathodic treatment and substantially immediately immersing it in an aqueous copper bearing electrolyte and initiating electro-deposition of copper thereon by use of a plating current not exceeding 100 amperes per square foot of cathode surface.

13. The method of preparing a stainless steel surface of a cooking vessel for receiving a relatively thick, strongly adhering layer of electro-deposited copper which comprises roughening said surface, making the roughened surface a cathode in a non-metal bearing aqueous sulphuric acid electrolyte to subject it to electrolytically released hydrogen without depositing metal thereon, and removing the vessel from said electrolyte upon the completion of the cathodic treatment and substantially immediately immersing it in an aqueous sulphuric acid copper sulphate electrolyte having, by weight, 5 to 15% sulphuric acid and 15 to 25% copper sulphate with the amount of sulphuric acid greater than the amount of copper sulphate and initiating electro-deposition of copper thereon by use of a plating current not exceeding 100 amperes per square foot of cathode surface.

14. The method of coating a stainless steel surface of a cooking vessel with a strongly adhering layer of copper which comprises preparing the surface for receiving such coating by roughening it and making the roughened surface a cathode in a non-metal bearing aqueous sulphuric acid bath to treat it with electrolytically released hydrogen without depositing metal on it; and forming the copper layer by first electro-depositing a strike coating of copper on the roughened, cathodically treated surface, and then depositing the remainder of the copper layer on said strike coating; the forming of the strike coating comprising removing the roughened surface from the

non-metal bearing electrolyte upon the completion of the cathodic treatment and substantially immediately immersing it in an aqueous copper bearing electrolyte and initiating electro-deposition of copper thereon to deposit the strike coating by use of a plating current not exceeding 100 amperes per square foot of cathode surface; the forming of the remainder of the copper layer comprising electro-depositing a relatively thick layer of copper on the strike coating by use of an aqueous sulphuric acid copper sulphate electrolyte having, by weight, 5 to 15% sulphuric acid and 15 to 25% copper sulphate, with the amount of sulphuric acid less than the amount of copper

sulphate, and a plating current of greater density than the first mentioned plating current but not exceeding 500 amperes per square foot of cathode surface.

5 15. The method according to claim 14 in which the vessel is axially rotated during the plating of both the strike coating and the thick layer, and at such speed during at least the plating of said layer as to draw an attenuated film of electrolyte up the adjacent side walls of the vessel above the normal level of the electrolyte.

JAMES M. KENNEDY.  
ARTHUR P. KNIGHT.  
HAROLD J. LEE.